

# UNITED STATES PATENT OFFICE.

JOHANN F. E. SCHULTZE, OF POTSDAM, PRUSSIA, ASSIGNOR TO HIMSELF  
AND H. M. C. WERNICH, OF WASHINGTON, DISTRICT OF COLUMBIA

## IMPROVED GUNPOWDER.

Specification forming part of Letters Patent No. 38,789, dated June 2, 1863.

*To all whom it may concern:*

Be it known that I, JOHANN FREDRICH EDWARD SCHULTZE, of the Kingdom of Prussia, have invented a new and improved explosive powder, applicable to the purposes to which ordinary gunpowder is applied; and I do hereby declare that the following is a full and exact description thereof, of the elements of its composition, and of the process of its manufacture.

The fundamental element of the explosive compound is wood, or, perhaps, more properly speaking, woody fiber, which, after due mechanical and chemical treatment, is converted into this compound. In the first step of this manufacture I take any species of wood—such as poplar, linden, ash, oak, &c.—in the form of logs or boards, and divide them up, by sawing or otherwise, into thin sheets or veneers. The harder kinds of wood make a more explosive powder, and therefore the best for the manufacture of that kind used for mining purposes.

The manufacture of this powder as a whole may be very appropriately divided into three processes, sufficiently distinct in themselves for distinctive description, and to be described under their several heads.

I. *Mechanical preparation of the material.*—As before remarked, the wood to be used is to be reduced, by sawing or otherwise, to thin sheets or veneers of about the one-sixteenth of an inch in thickness when the powder to be made is for ordinary small-arms. As the thickness of these plates or veneers determines the size of the grain of the powder, this thickness may be lessened or increased to suit the grains to the purposes to which the powder is to be applied. These plates or veneers are then passed under or through a punching-machine—such, for instance, as is used in the manufacture of cards. The diameter of the punches should be about the same as the thickness of the plates or veneers, as this gives a regularity of structure to the granular mass of the powder. I do not deem it necessary to describe the machinery necessary for this purpose, as it constitutes no part of my invention, and any good mechanic can readily construct one sufficient for the accomplishment of this simple operation. The cyl-

inders of the wood thus formed constitute the part to be used in the further processes for the manufacture of the best kind of powder. The reticulated plates or veneers of wood left by the punching operation can now be utilized by cutting them up into small fragments. The plan I have adopted and found to answer very well is to pass the reticulated plates or veneers through rollers furnished with cutters around the periphery and at about one-eighth of an inch from each other. When passed through such rollers the plates or veneers will be cut into strips of the width, of course, of the space between the cutters—that is, this would be the case if one set of rollers only were used; but I find the better plan to be to pass a cutting-roller over the plates or veneers in one direction and another across them in a line at a right angle to the former. I thus cut the whole plate or veneer at once, as it were, into the desired form. The material thus produced can be advantageously used for the preparation of such powder as is used in fortifications and the navy, but is not so well adapted to land service, as the irregularities in the form of the grains render them liable to injury from abrasion. If I adopt the first plan suggested for cutting these reticulated plates or veneers into strips—that is, by passing them through rollers with cutters—I still adopt the plan mentioned or some other for cutting them transversely, that the whole may be reduced to the condition of a coarse irregular-grained powder.

II. *Chemical treatment of the granulated woody material.*—The chemical treatment of the grains produced by the foregoing operation to convert them into the explosive powder may be advantageously described under the following heads: first, the removal of acids and other easily-soluble substances; second, the removal of the proteine, albumen, &c.; third, the removal of the coloring-matters; fourth, submission of the grains to the action of nitric acid; fifth, saturation of the grains with salts containing oxygen and nitrogen.

1. *The removal of acids and other easily-soluble substances.*—Into a kettle, which I prefer to be of copper and of a suitable size, is to be put as much water holding three pounds of carbonate of soda in solution as will freely float

one hundred pounds of the grains prepared as described under head I. This amount of the grain being introduced and stirred up with the alkaline solution, the whole is boiled together for three or four hours. At the end of this time the liquid, becoming discolored, is removed and a fresh supply added and the boiling continued for three or four hours more. The grains are then removed and exposed for twenty-four hours to a current of fresh and cold running water.

2. *Removal of the proteine, albumen, &c.*—The grains from the operation 1, having been dried, are placed in boxes of sheet-iron or other proper material having a colander or sieve like bottom and steam passed through them for about fifteen minutes. The proteine and albumen are thus separated and pass off with the water of condensation from the steam. After this the grains are again placed in cold fresh and running water for about twenty-four hours, and then dried.

3. *The removal of the coloring-matter.*—This might perhaps with equal propriety be called the "bleaching process." To accomplish this purpose the grains may be treated with a solution of chloride of lime, or with chlorine gas. If chloride of lime be used, about fifteen pounds of the salt is dissolved in about two hundred and sixty (260) pints of water in an air-tight vessel. The dried grains from operation 2 are placed in another vessel and so much of the solution of the chloride poured into it as will entirely cover the grains. After about two hours, keeping the grains constantly stirred during the time, the process will be finished. The grains are then removed from the solution and washed with cold fresh running water, after which they are placed in water which is to be brought up to the boiling-point and then removed and again placed in cold fresh running water for about twenty-four (24) hours, after which they are to be dried at a moderately-high temperature. When chlorine gas is used the grains from operation 2 are placed in a proper vessel and the gas passed freely through them until the discoloration is accomplished. They are then subjected to the washing described above, when the chloride solution is used and then dried.

4. *Submission of the grains to the action of nitric acid.*—As a preliminary step in the operation, forty (40) parts, by weight, of concentrated nitric acid of a specific gravity of 1.48 to 1.50 are mixed with one hundred (100) parts, by weight, of concentrated sulphuric acid of specific gravity of 1.84, the mixture of the acid to be constantly stirred or agitated for about two hours, when it is to be set aside in some cool place for use. Then in an iron or other suitable vessel, around which cold water should be kept constantly circulating, or by some other appropriate arrangement the vessel should be constantly subject to a refrigerating process, one hundred parts, by weight, of these mixed acids are placed, and six (6) parts, by weight, of the grains gradually added, stirring the

whole constantly for two or three hours, at the end of which time the operation will be completed. The grains are then separated from the adhering acid by draining them into a centrifugal machine, or by any other process capable of accomplishing the same purpose. The centrifugal apparatus I prefer, as it is well known that moisture can by the action of this machine be promptly and successfully removed. As this machine is well known and used in sugar-refineries, laundries, &c., a description of it is not deemed necessary. The grains removed from the centrifugal machine are again placed in cool fresh running water for two or three days; then again boiled up in a weak solution of carbonate of soda and again exposed for twenty-four hours to cool fresh running water and then dried. This brings the grains to a state in which they may be stored away for the final operation, or they may be proceeded with at once, as follows:

5. *Saturation of the grains with a salt or salts containing oxygen and nitrogen.*—The salts used in this operation are nitrate of potassa (salt-peter) and nitrate of barytes. The two may be used together, or the former (nitrate of potassa) alone. When both salts are used a solution of them is made by dissolving 22.5 parts of the nitrate of potassa and 7.5 parts of the nitrate of barytes in two hundred and twenty parts of water at 112° Fahrenheit and stirring up in it one hundred parts of the grains, prepared as above described, for ten or fifteen minutes. When only the one salt (nitrate of potassa) is used dissolve twenty-six parts thereof in the above amount (two hundred and twenty parts) of water at 67.5° Fahrenheit and treat one hundred parts of the grains in the same manner as when both salts are used. The grains having thus been subjected to the action the salt or salts containing nitrogen and oxygen in their composition are removed to a room or chamber having the temperature in its air kept at from 90° to 112° Fahrenheit, where they should remain from twelve to eighteen hours to be thoroughly dried. After this they are dusted by means of a drum or screen. The process is then completed and the powder ready for use. The numbers given in the preceding description have been found to give the best results and to yield a powder of the finest qualities; but it is not to be understood that my invention requires a rigid adherence to them in carrying it out; on the contrary, many changes may be made without departing from its spirit or affecting the principles upon which it is founded. If it is desired to avoid the dangers of transportation to which all such explosive compounds are exposed, the final process, as described under 5, Sec. II, may be delayed and the materials themselves—that is, the grains of 4—and the salts or their solutions (nitrate of potassa and nitrate of barytes) transported to the place at which the powder is required and the final process completed there. As neither the grains nor the salts separately are explosive we avoid all causes of danger

and apprehension from the most difficult transportation over the most distant roads by this means.

*III. Utilizing the dust from the sifted powder.*—The dust produced by the several operations as described amounts sometimes to ten or twelve per cent. of the whole mass. To utilize this powder or dust it is mixed into a paste with water or gum-water and rolled or spread out into sheets of about three-eighths of an inch in thickness. These sheets are then put under a powerful hydraulic or other press and reduced to the thickness of the plates or veneers described in the first part of this specification—that is, about the one-sixteenth ( $\frac{1}{16}$ ) of an inch. These sheets are then punched in the same way as the plates or veneers and the grains dried. The powder produced by this operation on the dust is the best for rifled small-arms.

The following may be stated as the leading advantages which this explosive compound possesses over the ordinary gunpowder:

First. It has for equal weights from three to four times the strength of gunpowder, while its weight is only about one-third.

Second. It can be manufactured at less cost than gunpowder.

Third. Its explosive effect is more regular than gunpowder in consequence of the greater uniformity in the size and character of its grains.

Fourth. Its volatile products, being chiefly oxygen, the vapor of water, nitrogen, and a small quantity of carbonic acid, are not offensive to the lungs, while those from gunpowder are well known to be exceedingly so. The volatile products from my powder are lighter than atmospheric air and quickly disappear. In

ordinary gunpowder it is the reverse. In case-mates, iron-clad steamers, mines, &c., this is an important difference.

Fifth. It soils the gun or cannon in the slightest possible degree—indeed almost to an inappreciable extent—owing, no doubt, to the removal by the treatment of the grains of almost or quite all metallic or earthy matters from the wood and the complete combustion of all the elements of the powder.

Sixth. It admits of being manufactured in such a way that it may be stored or transported without any danger from explosion.

Having thus fully explained the nature, character, and mode of preparing my invention, what I claim therein, and desire to secure by Letters Patent of the United States, is—

1. The production of grains or particles from plates, sheets, or veneers of wood, substantially in the manner set forth.

2. The preparation of these grains or particles of woody substance, substantially in the manner set forth, for conversion into an explosive powder.

3. Combining the grains or particles of wood or woody substance thus prepared with salts containing oxygen and nitrogen in their composition for the production of an explosive powder, substantially as set forth.

4. The preparation of the dust or fine powder resulting from the preceding operations for the production of an explosive powder.

5. The granulated explosive powder produced by the process hereinbefore described.

JOHANN FREDRICH EDUARD SCHULTZE.

Witnesses:

WALTHER BAUENDAHL,  
W. V. SCHULTZ.